

Dec. 15, 1964

E. M. LEACH

3,160,931

CORE CASTING METHOD

Filed Jan. 3, 1961

3 Sheets-Sheet 1

FIG. 1



INVENTOR.

EDWARD M. LEACH  
BY

Leo A. Plum, Jr.

ATTORNEY

Dec. 15, 1964

E. M. LEACH

3,160,931

CORE CASTING METHOD

Filed Jan. 3, 1961

3 Sheets-Sheet 2



FIG. 2



FIG. 4



FIG. 3

INVENTOR.  
EDWARD M. LEACH

BY

Leo A. Plum, Jr.  
ATTORNEY

Dec. 15, 1964

E. M. LEACH

3,160,931

CORE CASTING METHOD

Filed Jan. 3, 1961

3 Sheets-Sheet 3



1

3,160,931

## CORE CASTING METHOD

Edward M. Leach, Bunker Hill, Ind., assignor to Union Carbide Corporation, a corporation of New York  
Filed Jan 3, 1961, Ser. No. 80,292  
6 Claims. (Cl. 22—194)

This invention relates to an improvement in metal casting methods and in particular to providing preformed cores for forming internal passages and hollow areas in metal castings.

In the precision casting of metallic articles in ceramic molds, internal passages in the castings are formed through the use of ceramic cores placed in the mold, or where cores are not suitable, by drilling and machining the finished casting to form the passages. The use of cores to form such internal passages in castings is preferred over drilling or other metal working operations because of the greater expense of the latter methods. However, because of the small size and intricate configuration of many proposed internal passages in castings, workable cores can not be produced of the needed size and shape with the result that the passages must be drilled out or the design of the casting changed to fit present day core-making capabilities.

In one precision casting process, the shell mold casting process, a pattern of the object to be cast is made in wax or plastic. Any cores needed to form internal passages in the article are embedded in the wax pattern in their proper location. The wax pattern and core assembly is then coated with a shell by dipping the assembly repeatedly into slurries of refractory binders followed by a stuccoing with refractory particles. The cores are designed to protrude from the wax pattern in places so that these ends of the cores are anchored into the shell. A shell of sufficient thickness, usually from  $\frac{1}{4}$  to  $\frac{5}{8}$  inch, is built up around the wax pattern, and the mold is then fired to hardness—the wax material melting or burning out, leaving a cavity in the shell of the desired configuration complete with cores to form internal passages in the casting. It is easy to see that the cores are the weakest part of this shell mold for the strength of the shell mold itself is easily built up by increasing the thickness of the mold while the cores are of unchangeable dimensions—being of the thickness and width of the proposed internal passageway. For this reason the design problems in regard to the shell mold compositions and processes are quite different from those problems involved in designing suitable core compositions and forming processes.

The compositions used to make the cores must be such as to give a high strength to the core, even in thin sections, and be capable of producing smooth finishes on the cores.

Besides the need for a core material having the necessary strength and surface forming qualities, the process of fabricating the cores must be such as will easily fit into production line operations. There are several core forming processes of which two are outlined below.

Where a large number of castings are to be made, a metal die of the proposed core shape needed is produced. Then a substantially dry ceramic core material is pressure cast in this die. The die injection must be done under pressure to eliminate voids and to compress the material to a proper strength with the result that the expensive metal dies are worn down by the abrading ceramic material.

Where the small number of castings involved does not justify the expenses of metal dies, another core-forming process can be used with plastic, rubber, or ceramic dies. Because of the low strength of such dies, pressure casting

2

methods cannot be employed and, instead, the ceramic core material is prepared in the form of a free-flowing slurry and is poured into the dies. After the core material hardens within the die, it is removed. The hardening time may vary from about 35 to 70 minutes, depending on the composition of the slurry material. This constitutes a series drawback to production economy, because only about 10 cores can be produced from each die per 8 hour day. The mere provision of a quick-setting material affords no improvement in the process because such quick-setting materials must be used when made, having little or no shelf-life—another property required of materials used in production line operations.

It is the primary object of this invention, therefore, to provide a ceramic composition suitable for forming intricate cores of high strength and smooth surface finish.

It is another object of this invention to provide a process for forming cores of the type described which process is simple and amenable to production line operations.

Other aims and advantages of this invention will be apparent from the following description and the appended claims.

In the drawings:

FIG. 1 is a flow-chart of the core-forming process of this invention;

FIG. 2 is a perspective view of a large turbine stator blade of double-curvature containing three long, thin blade-like cores forming the internal passages;

FIG. 3 is a perspective view of a small turbine blade containing an intricate core assembly;

FIG. 4 is a perspective view of the core assembly shown in the blade of FIG. 3;

FIG. 5 is a chart showing the relationship of gelation or hardening time of the core material and the die temperature in the forming of the cores by the process of this invention.

In accordance with the objects a process for forming ceramic castings is provided comprising preparing a liquid binder solution consisting essentially of alcohol, ethyl silicate solution, hydrochloric acid and water, mixing with said liquid binder solution a refractory particle and binder solids mix consisting essentially of inert refractory particles, powdered feldspar, powdered lead borate glass frit, and magnesia, casting the resulting slurry at a slurry temperature no higher than room temperature in a die having a temperature from about 90° F. to about 140° F., removing the solidified casting from the die and firing it to hardness at a temperature between 1700° F. and 2400° F. for from 1 to 4 hours.

The proper control of temperature promotes a fast gelation of the slurry. By casting this slurry composition in a die heated to a temperature from 90° F. to 140° F., a much faster gelation of the slurry occurs than the 35 to 70 minute gelation time of some other slurry compositions in other processes. The temperature of the slurry should be no higher than room temperature—room temperature here meaning the temperature slurry would take on after preparation if allowed to stand, usually room temperature. As will be seen from FIG. 5 of the drawing, the use of a chilled slurry, i.e., at a temperature less than room temperature, in a heated die gives a faster gelation time.

It is also necessary to chill the slurry where it is not to be used immediately after preparation. The mixing of the constituents of the liquid solution causes an exothermic reaction that raises the temperature of the liquid solution to about 130° F. The solids mix is not added to the liquid solution at this temperature or gelation would start to take place uncontrollably in less than an hour. Therefore the liquid solution is preferably

aged for about 12 hours and chilled to a temperature between  $-10^{\circ}$  F. and  $20^{\circ}$  F. before the solids mix is added. The resulting slurry of liquid solution and solids mix is preferably itself chilled to a temperature between  $-10^{\circ}$  F. and  $20^{\circ}$  F. until used. The slurry is generally cast at a temperature between  $10^{\circ}$  F. or  $20^{\circ}$  F. and room temperature, which is generally no higher than  $80^{\circ}$  F.

More specifically, as is shown in FIG. 1, a process for forming ceramic cores for use in casting molds is provided comprising preparing at room temperature a liquid binder solution consisting essentially by weight of from about 35 percent to 75 percent alcohol, from about 65 percent to 25 percent ethyl silicate solution, from about 4 percent to 12 percent water and from about 0.2 percent to 0.6 percent concentrated hydrochloric acid, reducing the temperature of the liquid binder solution to a temperature between  $-10^{\circ}$  F. and  $20^{\circ}$  F. and mixing therewith a refractory particle and binder solids mix consisting essentially by weight of from 6 percent to 9 percent powdered feldspar, from about 1.5 percent to 3.5 percent powdered lead borate glass frit from about 0.05 percent to 4.5 percent magnesia and the balance substantially all particulated refractory materials selected from the group consisting of silica, alumina, zircon, and firebrick grog, the amount of solids mix and liquid solution being about 70 percent to 85 percent by weight solids mix and the balance liquid solution, casting the resulting slurry at a slurry temperature no higher than room temperature in a die having a temperature from about  $90^{\circ}$  F. to  $140^{\circ}$  F., removing the solidified core from the die and firing it to hardness at a temperature between about  $1700^{\circ}$  F. and  $2400^{\circ}$  F. for from 1 to 4 hours.

The composition of the slurry is designed to produce ceramic cores of high green strength (strength before firing, necessary for normal handling of the article after casting and before firing) as well as high fired strength, surface and dimensional quality, and inertness to the metals and alloys being cast.

A preferred liquid solution contains by weight from 48 to 54 percent alcohol, from 39 to 45 percent ethyl silicate solution, from 5.5 to 7.5 percent water, and from 0.3 to 0.5 percent concentrated hydrochloric acid. A typical liquid solution contains 51 percent by weight isopropyl alcohol, 42 percent by weight ethyl silicate grade 40, 6.6 percent by weight water, and 0.4 percent by weight concentrated hydrochloric acid. The specified proportions of alcohol and ethyl silicate provide the low temperature binders while the water and acid coat as the gelation time control agents and the hydrolysis catalyst, respectively. Ethyl silicate grade 40 is generally used, containing about 40 percent by weight  $\text{SiO}_2$ . Other grades of ethyl silicate may be used provided they contain at least 28 percent by weight  $\text{SiO}_2$ . Common commercial denatured alcohol and in particular isopropyl alcohol is recommended. However other similar solvents may be used. Hydrochloric acid is preferred but other mineral acids may be used.

While the ethyl silicate content provides a low temperature binder for green strength, the solids mix contains feldspar and lead borate glass frit for high temperature bonding.

The high temperature binder feldspar, which is added as a powder, is present in amounts from 6 to 9 percent by weight. The high temperature binder lead borate glass frit, also added as a powder, is present in amounts from 1.5 to 3.5 percent by weight. From 0.05 to 4.5 percent by weight magnesia of a particle size less than 200 mesh is added to the solids mix to neutralize acids and establish a slurry pH at least about 7, thereby promoting gelation of the slurry.

The balance of the solids mix contains refractory particles in specified particle sizes and of the following materials: zircon, silica, alumina, and firebrick grog. Of

special importance in producing the smooth-surfaced yet strong core castings of this invention is the inert nature of the selected refractory material and the range of refractory particle sizes. The refractory materials used, zircon, silica, alumina, and firebrick grog are all chemically inert manufactured fused products which have no inherent bonding characteristics. It is important that these materials be chemically inert and without inherent bonding characteristics so that there is no danger of interaction with the metal being cast or with the binders in the slurry. While the above-listed refractory materials are all generally nonreactive with the ordinary metals cast, there are some general rules to be followed in selecting the refractory base of the slurry, for example: (1) in casting alloys that contain an appreciable amount of aluminum, zircon or alumina base cores are used; and (2) in casting alloys that contain an appreciable amount of manganese, silica-base cores should not be used.

The particle size distribution of the refractory materials are based on a blend of at least two different ranges of average particle size. The use of these blends guarantee a casting which is substantially lower in voids than when only one size range of particle is used in the slurry. The absence of large numbers of voids accounts for a smoother core surface because of the absence of surface depressions caused by voids or spaces between large particles.

It is to be noted that in the manufacture of molds using slurries and refractory particles, it is common to produce smooth surfaces by decreasing the particle size of the refractory materials. In the case of shell molds the particle size of those layers which will be adjacent the metal are maintained small to provide a smooth surface while the outer layers are formed with larger particles to give strength. While such a procedure is acceptable with a shell mold or investment mold because the mold thickness can be of unlimited size, it would not necessarily work with a small core casting which must have strength as well as smoothness in a limited and uniform cross-section. Therefore a blend of small and large particle sizes is generally used. The broad and narrow ranges for these particle size distributions are given below in Table I for each of the refractory materials. Also given is a typical solids mix composition, it being understood that the exact compositions are selected from the broad ranges in accordance with such considerations as the configuration, size and weight of the individual core. The particle sizes referred to are of the standard Tyler Sieve Series.

TABLE I

Solids Mixes

|                                       | Broad       | Preferred | Typical Composition |
|---------------------------------------|-------------|-----------|---------------------|
| Zircon-Base Solids Mix:               |             |           |                     |
| Zircon Flour (-200 Mesh)              | 30 to 70    | 45 to 55  | 50.5                |
| Zircon Sand (-80 +200 Mesh)           | 70 to 30    | 35 to 43  | 38.25               |
| Magnesia (-200 Mesh)                  | 0.05 to 4.5 | 1.5 to 2  | 1.25                |
| Lead Borate Glass Frit (powder)       | 1.5 to 3.5  | 1.5 to 3  | 2.5                 |
| Feldspar (powder)                     | 6 to 9      | 6 to 8    | 7.5                 |
| Silica-Base Solids Mix:               |             |           |                     |
| Silica Flour (-68 Mesh)               | 22 to 60    | 30 to 40  | 35                  |
| Silica Flour (-100 Mesh)              | 50 to 20    | 34 to 44  | 39                  |
| Silica Flour (-325 Mesh)              | 8 to 15     | 10 to 13  | 12.25               |
| Magnesia (-200 Mesh)                  | 0.05 to 4.5 | 1.5 to 2  | 1.75                |
| Lead Borate Glass Frit (powder)       | 1.5 to 3.5  | 1.5 to 3  | 2.5                 |
| Feldspar (powder)                     | 6 to 9      | 6 to 8    | 7.5                 |
| Alumina-Base Solids Mix:              |             |           |                     |
| Powdered Alumina (-60 Mesh)           | 42 to 68    | 50 to 60  | 55                  |
| Powdered Alumina (-35 Mesh)           | 22 to 12    | 14 to 20  | 17                  |
| Crushed Firebrick Grog (-28 +50 Mesh) | 12 to 22    | 14 to 20  | 17                  |
| Magnesia (-200 Mesh)                  | 0.05 to 4.5 | 1.5 to 2  | 1.75                |
| Lead Borate Glass Frit (Powder)       | 1.5 to 3.5  | 1.5 to 3  | 2.5                 |
| Feldspar (Powder)                     | 6 to 9      | 6 to 8    | 7.5                 |

TABLE I—Continued

|                                       | Broad       | Preferred | Typical Composition |
|---------------------------------------|-------------|-----------|---------------------|
| Firebrick Grog-Base Solids Mix:       |             |           |                     |
| Crushed Firebrick Grog (-10 +48 Mesh) | 10 to 30    | 15 to 25  | 20                  |
| Crushed Firebrick Grog (-50 Mesh)     | 20 to 50    | 30 to 40  | 35                  |
| XXX Silica Flour (-325 Mesh)          | 20 to 60    | 40 to 50  | 45                  |
| Magnesia                              | 0.05 to 4.5 | 1.5 to 2  | 1.75                |
| Lead Borate Glass Frit (Powder)       | 1.5 to 3.5  | 1.5 to 3  | 2.5                 |
| Feldspar (Powder)                     | 6 to 9      | 6 to 8    | 7.5                 |

15

The amount of solids mix added to the liquids mix to form the slurry is broadly from about 70 percent to 85 percent by weight solids mix and the balance liquids mix. A preferred relationship is 77 percent by weight solids mix and the balance liquids mix for the zircon-base mix and the following percents by weight solids mix for the other refractory bases: silica-base, 72 percent; alumina-base, 80 percent; firebrick grog, 83 percent.

As an example of the practice of the invention a liquid binder mix was prepared by mixing at room temperatures 51 percent isopropyl alcohol, 42 percent ethyl silicate grade 40, 6.6 percent water, and 0.4 percent concentrated hydrochloric acid. The combination of these ingredients effects an exothermic reaction that increase the temperature of the mix to about 130° F. The mix is agitated until this maximum temperature is reached after which the liquids mix is allowed to cool to room temperature and aged for about 12 hours at room temperature. If the slurry is to be used immediately, the solids mix is now added to the liquids mix. If, however, the slurry is not to be used within about one hour after preparation, as was the case in this example, then the liquids mix is cooled to about 10° F. after aging. The solids mix is added to the chilled liquids mix and stirred for about 5 to 10 minutes and then the slurry is chilled to a temperature from -10° F. to +20° F. until used. The solids mix was zircon-based and consisted of 50.5 percent zircon flour (-200 mesh), 38.25 percent zircon sand (-80 +200 mesh), 1.25 percent magnesia (-200 mesh), 2.5 percent lead borate glass frit (powder), and 7.5 percent powdered feldspar. About 77 percent by weight solids mix was added to 23 percent liquids mix.

Dies were prepared of the core shapes to be cast which were similar to those shown in FIGS. 2, 3 and 4. Since the casting method did not involve pressure casting, the dies could be made of rubber, plastic, ceramic or glass. The dies here were made of an epoxy resin. The slurry had a temperature of about 10° F. at the time of casting and the die had a temperature of about 140° F. Gelation occurred almost immediately. The core was removed from the mold and fired at 2000° F. for about 2 hours. This firing cycle of 2 hours at 2000° F. is the preferred cycle.

It is to be noted that the slurry need not be used immediately after preparation, but may be stored for a considerable period of time at a temperature between -10° and 20° F. Ordinarily the slurry will gel and harden at room temperature in about one hour; however, at about 10° F. the slurry remains fluid and usable for at least 240 hours. Because of this property, large batches of slurry may be prepared in advance and stored until needed, instead of the normal practice of preparing a smaller batch every hour. This feature contributes to improved continuous mass production operations at a lower cost and insures uniformity of product.

The gelation time of the slurry is a function of the heat transfer characteristics of the die-slurry system. In a series of tests to determine the effect of temperature on

the gelation time, the temperatures of the die and slurry were varied and all other known variables were kept constant, i.e., mass, volume, configuration and composition. By fixing these variables the specific heat, thermal conductivity and coefficient of heat transfer of the die and slurry are also held constant. The heat transfer from die to slurry is a direct function of the temperature difference. FIG. 5 shows the results of these tests. Note that the gelation time is in direct relationship with the temperature difference of the die-slurry system. Because of this relationship, the gelation time may be accurately controlled, thereby eliminating such variables as room temperature, humidity and so on. These ambient variables have a pronounced effect on gelation time of currently used materials and make continuous processing very difficult in the present art.

It is seen from FIG. 5 that the decrease in gelation time from the normal time of 35 to 70 minutes takes place when the die is at about 90° F. If the slurry is at 10° F. the normal storage temperature, then the slurry will gel in the 90° F. die in about 33 minutes. The gelation time shortens rapidly as the temperature difference is increased by increasing die temperature to 130° or 140° F. or increasing the slurry temperature slightly. The minimum die temperature for a 10° F. slurry would be 90° F. therefore. Generally the slurry will be warmer than 10° F. as a result of standing awaiting use. If the slurry is at 80° F. and the die at 100° F., the gelation time will be 18 minutes. As the die temperature is increased to about 130° or 140° F., the gelation time decreases rapidly. In general the die temperature for slurries having a temperature between 10° F. and 80° F. will preferably be between about 100° F. and 140° F. The gelation time will be shortest when the temperature difference is the greatest, i.e., when the die temperature is 130° F. or 140° F. A specific die temperature can be selected which suits the needs of the specific production line involved. This depends on the temperature of the slurry and speed required in producing castings. By using a die temperature between 120° F. and 140° F. almost immediate gelation can be effected.

The casting of the slurry compositions in the heated die causes a "coring" effect which improves surface quality of the cores. When the slurry is poured into the heated die, the sudden temperature change effects a rapid gelation of the slurry that is immediately adjacent to the inner wall of the die. If present, any evolution or accumulation of gas bubbles will converge toward the center of the slurry mass and will not form on the surface of the finished core where they would cause irregularities.

The storage of the slurry for comparatively long periods of time does not effect the gelation or hardening time of the slurry except within the small ranges shown in Table II. A freshly made slurry will gel in about the maximum time as shown in the ranges, while an aged slurry will gel in about the minimum time. Aging at 10° F., then is seen not to greatly affect the properties of the slurry.

TABLE II

## Effect of Temperature on Gelation Time

| Condition | Die Temp., ° F. | Slurry Temp., ° F. | Temp. Difference | Gelation Time, min. |
|-----------|-----------------|--------------------|------------------|---------------------|
| A         | 80              | 10                 | 70               | 35 to 50            |
| B         | 130             | 10                 | 120              | 3 to 5              |
| C         | 80              | 80                 | 0                | 25 to 30            |
| D         | 130             | 80                 | 50               | 2 to 6              |

Conditions A and B as shown in Table II represent slurries that were cooled to 10° F. before casting. Con-

ditions C and D represent slurries that were used at room temperature.

It is to be noted that the slurry temperature should not be higher than the die temperature. If the slurry is used at a higher temperature than the die, the gelation time will be prolonged to an undesirable degree and will be more difficult to control.

By providing the above described process for casting this class of materials, applicant has made it possible to accurately predict and control a convenient gelation rate that will promote rapid and efficient production as well as good quality control and lower production costs.

The slurries produced according to the specifications above can be cast into core shapes of the most intricate configurations. The core shapes have sufficient green strength after casting to maintain themselves during further handling. After firing, the cores are strong enough to withstand rough handling and can be used in pressure casting methods. The cores are compatible with the liquid metal, have a low and uniformly predictable rate of thermal expansion, and are readily removed from the casting by chemical means, sand blasting, etc.

In FIGURES 2, 3 and 4 two cores are shown which were produced by the process of this invention. FIG. 2 shows a wax pattern and ceramic core assembly 11 for use in making a turbine stator blade. Three cores 12, which were produced according to this invention are embedded in the wax pattern 13 of the blade to form three coolant passageways in the blade. To make a mold this assembly is coated with a slurry of liquid binders and refractory powders and then stuccoed with larger refractory particles. This process can be repeated until a multi-layer shell mold of sufficient thickness is built up around the assembly 11. The ends of the three cores 12, extending out of the wax pattern, are now embedded in the shell mold so that on removal of the wax pattern 13 by melting or dissolving, a cavity is left in the mold with the three ceramic cores properly positioned therein. After the mold is fired, molten metal may be poured in forming a blade of the same configuration as the original wax pattern except that the cores 12 are removed leaving the internal passages in their place. The blade shown in FIG. 2 is about 6 and 1/2 inches high and has a curved airfoil-shaped cross section. The cores are each about 6 inches long, 1 and 1/4 inches wide at the tip and have a thickness varying from 1/16 to 1/8 inch. These cores all have the same curves and twist as the airfoil shaped blade. Previously blades of this size and shape could not be made by the "lost wax" process because cores of such a length and thinness could not be made strong and smooth enough. To make such a blade, sheet stock was formed around spaced ribs (the coolant passages being the spaces between the ribs) and welded together. With the compositions and processes of this invention, cores are now producible thereby making possible the more rapid production of this type blade.

In FIGURES 3 and 4 another form of core is shown which also could not be produced successfully until the advent of this invention. FIG. 4 shows a wax pattern and core assembly 14 of a small turbine blade about 1 inch wide and about 2 inches high. The core assembly 15 of FIG. 3 is shown embedded in the wax pattern 16. This fork-shaped core assembly 15 represents the intricate arrangement of coolant passages in the blade (shown as dotted lines in the wax pattern of FIG. 4.). The small vertical holes in the airfoil section of the blade have a diameter of only 0.030 inch and are usually formed by drilling of the casting rather than by the use of cores.

The core assembly 15 is made up of a T-shaped section 17 which is cast with the slurries described above with four holes 18 in the cross-bar 19 and fired to hardness. Quartz rods 20 of the proper diameter are sealed in these holes to form the fork-shaped core assembly 15 which is then embedded in a wax pattern and the

whole structure coated with ceramic slurries and particles to form a mold. When the wax pattern is melted out the core assembly remains firmly anchored in the walls of the mold. Prior art attempts to cast such coolant passages with composite quartz-ceramic cores were unsuccessful because of the low strength of the cores and the failure of assembly at the ceramic-quartz joint. It was necessary to cast a solid blade and then to drill out the internal passages.

It is to be noted that while the compositions and processes of this invention have been described in terms of the shell molding art and investment casting art, that the core forming compositions and processes of this invention can be used in other precision casting processes as well as in said casting and other founding methods.

What is claimed is:

1. A process for forming ceramic cores for use in casting molds comprising preparing a liquid binder solution consisting essentially by weight of from about 35 percent to 75 percent alcohol, from about 65 percent to 25 percent ethyl silicate solution, from about 4 percent to 12 percent water and from about 0.2 percent to 0.6 percent concentrated hydrochloric acid, reducing the temperature of the liquid binder solution to a temperature between -10° F. and 20° F. and mixing therewith a refractory particle and binder solids mix consisting essentially by weight of from 6 percent to 9 percent by weight powdered feldspar, from about 1.5 percent to 3.5 percent powdered lead borate glass frit, from about 0.05 percent to 4.5 percent magnesia and the balance substantially all particulated refractory materials selected from the group consisting of zircon, silica, alumina, and firebrick grog, the amount of solids mix and liquid solution being from about 70 percent to 85 percent by weight solids mix and the balance liquid solution, maintaining the resulting slurry at not greater than room temperature until used, casting the resulting slurry at a slurry temperature no higher than room temperature in a die having a temperature from about 90° F. to about 140° F., removing the solidified core from the die and firing it to hardness at a temperature between about 1700° F. and 2400° F. for from 1 to 4 hours.

2. A process for forming ceramic cores for use in casting molds comprising preparing a liquid binder solution consisting essentially by weight of from about 43 percent to 54 percent alcohol, from about 39 percent to 45 percent ethyl silicate solution, from about 5.5 percent to 7.5 percent water and from about 0.3 percent to 0.5 percent concentrated hydrochloric acid, reducing the temperature of the liquid binder solution to about 10° F. and mixing therewith a refractory particle and binder solids mix consisting essentially by weight of from 6 percent to 9 percent by weight powdered feldspar, from about 1.5 percent to 3.5 percent powdered lead borate glass frit, from about 0.05 percent to 4.5 percent magnesia and the balance substantially all particulated refractory materials selected from the group consisting of zircon, silica, alumina, and firebrick grog, the amount of solids mix and liquid solution being about 70 percent to 85 percent by weight solids mix and the balance liquid solution, maintaining the resulting slurry at a temperature between room temperature and about 10° F. until used, casting the slurry at a slurry temperature between 10° F. and room temperature in a die having a temperature from about 100° F. to 140° F. removing the solidified core from the die and firing it to hardness at a temperature between about 1700° F. and 2400° F. for from 1 to 4 hours.

3. The process of claim 2 wherein said selected refractory material is zircon and the amount of solids mix and liquid solution being about 77 percent by weight solids mix and the balance liquid solution.

4. The process of claim 2 wherein said selected refractory material is silica and the amount of solids mix and liquid solution being about 72 percent by weight solids mix and the balance liquid solution.

5. The process of claim 2 wherein said selected refractory material is alumina and the amount of solids mix and liquid solution being about 80 percent by weight solids mix and the balance liquid solution.

6. The process of claim 2 wherein said selected refractory material is firebrick grog and the amount of solids mix and liquid solution being about 83 percent by weight solids mix and the balance liquid solution.

## References Cited in the file of this patent

## UNITED STATES PATENTS

|           |                |                |
|-----------|----------------|----------------|
| 2,521,839 | Feagin         | Sept. 12, 1950 |
| 2,732,600 | Hanink et al.  | Jan. 31, 1956  |
| 2,818,619 | Bradley et al. | Jan. 7, 1958   |
| 2,892,227 | Operhall       | June 30, 1959  |
| 2,911,310 | Shaw et al.    | Nov. 3, 1959   |
| 3,032,425 | Leach          | May 1, 1962    |